

Nov. 20, 1962

H. HUG

3,065,073

METHOD FOR PRODUCING COMPOSITE BODIES OF ALUMINUM  
AND SINTERED ALUMINUM POWDER

Filed June 5, 1959

Fig. 1.



Fig. 2.



Fig. 3.



Fig. 4.



Fig. 5.



INVENTOR  
HANS HUG

BY

Morrison, Kennedy, Campbell  
ATTORNEYS

# United States Patent Office

3,065,073

Patented Nov. 20, 1962

1

3,065,073

## METHOD FOR PRODUCING COMPOSITE BODIES OF ALUMINUM AND SINTERED ALUMINUM POWDER

Hans Hug, Neuhausen am Rheinfall, Switzerland, assignor to Aluminium-Industrie-Aktien-Gesellschaft, Chippis (Switzerland), a joint-stock company of Switzerland

Filed June 5, 1959, Ser. No. 818,433

Claims priority, application Switzerland June 9, 1958  
8 Claims. (Cl. 75—208)

It is often desirable to have at disposal composite bodies which consist partly of wrought or cast aluminum or aluminum alloy and partly of sintered aluminum powder. This is especially the case with light metal pistons for engines. These pistons are exposed in service to high temperatures and are therefore made from heat-resisting alloys. Bodies made from sintered aluminum powder have proved to be very heat resistant. These sintered bodies are produced by powder metallurgy and are therefore more expensive than the usual wrought or cast alloys and, accordingly, for the reason of economy it is generally not practicable to make pistons wholly from sintered aluminum powder. In order to take advantage of the high heat-resistance of the sintered aluminum bodies efforts have already been made to make only those parts of the piston from sintered aluminum powder which are exposed to high temperatures, namely the piston head and the zone of the piston-rings, and to manufacture the other parts of the piston from wrought or cast aluminum alloys. For this purpose inserts made from sintered aluminum powder have been disposed in the body of the piston by casting or pressing. But it proved to be very difficult to obtain by these methods an intimate and unobjectionable bond between the insert and the surrounding parts of the piston.

It is an object of my present invention to eliminate the imperfection of the known methods and to produce composite bodies of aluminum and sintered aluminum powder with a satisfactory bond. In the following description the expression aluminum means unalloyed metal as well as aluminum alloys.

According to my invention aluminum powder is cold-pressed onto a conventionally-produced (wrought or cast) piece of aluminum, whereafter the composite body is heated and sintered under pressure (sinter-pressed).

The cold-pressing is preferably carried out in a die in which one introduces first the wrought or cast piece of aluminum and which is then filled with aluminum powder. The aluminum powder is suitably a flaky powder with an aluminum oxide content of at least 6% and a total grease content of less than 0.3%. Such a powder may be produced for example according to the method described in Patent No. 2,678,880 (British Patent No. 698,789, Japanese Patent No. 214,646), the aluminum oxide of the powder is formed during milling by oxidation of the powder particles and is not added as aluminum oxide powder to the aluminum powder.

The invention is described by way of example in the accompanying drawing, the figures showing different steps of the method. FIGS. 1 and 2 show in section the composite body before and after cold-pressing. FIG. 3 shows an engine piston obtained from a composite body made according to the invention. FIGS. 4 and 5 show in section the manufacture of a composite body with an annular insert before and after cold-pressing.

A cast or wrought piece 2 of aluminum or aluminum alloy (i.e. an "aluminum metal") is introduced into the die 1. Then the calculated amount of aluminum powder 3 is filled in. The press ram 4, for example the ram of a drop forge, compresses the powder at room temperature to the compact 5 which becomes thereby already bonded

2

to the piece 2. The cold-pressing is carried out under a pressure of for example 1 to 4 t./cm.<sup>2</sup>. The piece 2 in the FIG. 1 has an annular shoulder. But it is also possible to use a piece with an otherwise shaped or a flat bonding surface. The bonding surface may be provided for example with projections or grooves in order to increase the bonding area between both parts.

The cold-pressed body is then wrapped to aluminum foil, heated slowly in a furnace to the sintering temperature and sinter-pressed at this temperature under a pressure of for example 5 to 8 t./cm.<sup>2</sup>. One obtains in this way the desired dense structure of the sintered part and an intimate bond between it and the cast or wrought part 2.

15 The composite body may be shaped afterwards, by forging or otherwise, for example to the engine piston shown in FIG. 3. This piston consists of a wrought part 6 of aluminum alloy and of a heat resistant part 7 of sintered aluminum. The forging operation results in a 20 kneading of the whole body and increases especially the elongation of the sintered part of the composite piston.

FIGS. 4 and 5 show the way of applying an annular sintered part onto a cast or wrought body. In the die 1 a head piece 10 is placed on the cast or wrought body 8, 25 which has a projection 9. The aluminum powder 11 is filled in around this headpiece. For the cold-pressing one uses a hollow press ram 12 which produces the compact 13. From this cold-pressed body one may manufacture 30 by sinter-pressing and forging a piston having a piston-ring zone of sintered aluminum.

In the described examples the forging operation follows the sinter-pressing. But it is also possible to carry out the forging together with the sinter-pressing in one step.

For the manufacture of the sintered part one must consider the general working conditions for the making of sintered aluminum bodies (see, for example, the article "Sintered Aluminum Powder," by R. Irmann, Dr. Ing., appearing on pages 236-241 of Symposium on Powder Metallurgy, 1954, Special Report No. 58, published by 40 The Iron and Steel Institute, 4 Grosvenor Gardens, London, S.W. 1, and particularly the paragraph beginning "Melting point" in the right-hand column on page 238), but bearing in mind the properties of the cast or wrought part. If for example a sintered part must be bonded to a part made from an aluminum alloy, the sintering temperature must be below the lowest melting point of the alloy.

The cold-pressing of the composite body may be carried out by any process applying a sufficient pressure, not only by drop forging.

50 What I claim is:

1. A method of producing a composite body of sintered aluminum powder and an aluminous metal member formed originally by casting which comprises cold-pressing flaky aluminum powder under a pressure of not less than 1 t./cm.<sup>2</sup> onto said aluminous metal member, applying heat to the composite body thus produced to raise it to a sintering temperature below the melting point of the aluminous metal, and subjecting the composite body 55 to said sintering temperature under a pressure of not less than 5 t./cm.<sup>2</sup>.

2. A method as in claim 1 wherein the cold-pressing step is carried out at a pressure of from 1 to 4 t./cm.<sup>2</sup> and the sintering step is carried out at a pressure of from 60 5 to 8 t./cm.<sup>2</sup>.

3. The method according to claim 1, using a flaky aluminum powder having an aluminum oxide content of at least 6% and a total grease content of less than 0.3%.

4. The method according to claim 1, in which the cold-pressing is carried out in a die.

5. The method according to claim 1, in which the bond-

ing surface of the aluminous body is provided with grooves, in order to improve the bond.

6. The method according to claim 1, in which the bonding surface of the aluminous metal body is provided with projections.

7. The method according to claim 1, in which the composite body is thereafter forged.

8. The method according to claim 1, in which the cold-pressed body is subjected to sintering conditions under pressure by forging at high temperature.

## References Cited in the file of this patent

## UNITED STATES PATENTS

|           |                 |       |               |
|-----------|-----------------|-------|---------------|
| 1,950,356 | De Bats         | ----- | Mar. 6, 1934  |
| 1,989,186 | De Bats         | ----- | Jan. 29, 1935 |
| 2,044,853 | Laise           | ----- | June 23, 1936 |
| 2,549,596 | Hamilton et al. | ----- | Apr. 17, 1951 |
| 2,657,961 | Lassberg        | ----- | Nov. 3, 1953  |
| 2,796,660 | Irmann          | ----- | June 25, 1957 |
| 2,809,891 | Ennor           | ----- | Oct. 15, 1957 |

UNITED STATES PATENT OFFICE  
CERTIFICATE OF CORRECTION

Patent No. 3,065,073

November 20, 1962

Hans Hug

It is hereby certified that error appears in the above numbered patent requiring correction and that the said Letters Patent should read as corrected below.

Column 1, line 67, for "aluminum" read -- aluminous --;  
column 2, lines 54 and 55, for "pressinf" read -- pressing --;  
column 3, line 1, before "body" insert -- metal --.

Signed and sealed this 30th day of April 1963.

(SEAL)

Attest:

ERNEST W. SWIDER  
Attesting Officer

DAVID L. LADD  
Commissioner of Patents